# EUROPEAN PATENT SPECIFICATION

(11) **EP 0 881 277 B1**
(45) Date of publication and mention of the grant of the patent: **17.08.2005**
(21) Application number: 98304251.6
(22) Date of filing: 29.05.1998
(51) Int. Cl.: C10M 135/10, C10M 159/24

(54) **Use of metal sulfonates as friction modifiers**
Verwendung von Metallsulfonaten als Reibungsmodifiziermittel
Utilisation des sulphonates métalliques en tant qu'agents modifiant la friction

(30) Priority: 31.05.1997 JP 15792197; 31.03.1998 JP 10402198
(43) Date of publication of application: 02.12.1998
(73) Proprietor: TONEN CORPORATION, Chiyoda-Ku, Tokyo 100 (JP)
(72) Inventor: Taguchi, Shigeko, Kawagoe City, Saitama (JP); Ono, Megumi, Tachikawa City, Tokyo (JP); Tomizawa, Hirotaka, Tokorozawa City, Tokyo (JP)
(74) Representative: Dew, Melvyn John

(56) References cited:
- EP-A- 0 312 313
- GB-A- 2 182 948
- US-A- 3 910 994
- US-A- 4 225 446

## Description

### BACKGROUND OF THE INVENTION

### Field of the Invention

This invention relates to a friction modifier comprising a metal sulfonate and to a lubricating oil composition with the metal sulfonate added therein, and more specifically to a friction modifier comprising a metal sulfonate containing a specific chain hydrocarbon group and to a lubricating oil composition with the metal sulfonate added therein.

### Description of the Prior Art

From the need for resource and energy saving measures in all the industrial fields in view of environmental conservation, reductions in friction and wear through improvements in lubricating oils have also been investigated in the field of lubricating oils from a variety of viewpoints in recent years with a view to lowering fuel consumption rates. As a result, it has already become indispensable to incorporate additives in base stocks for lubricating oils so that the base stocks can be provided with desired friction characteristics. Accordingly, a number of friction modifiers have been proposed to date, resulting in the use of fatty acids and their metal salts, esters, amines and the like - all of which are of the oiliness improver type - and phosphate esters, phosphite esters, zinc dithiophosphate and the like - all of which are of the extreme pressure agent type - in wet brake oils, automatic transmission fluids, sliding surface oils, plastic working oils and the like and also in the use of phosphate esters, phosphite esters, acidic phosphite ester amine salts, molybdenum dithiophosphate, molybdenum dithiocarbamate and the like - all of which are of the extreme pressure agent type - in engine oils, gear oils, cutting oils and the like.

Meanwhile, an automatic transmission oil was disclosed, which had been obtained by adding magnesium sulfonate, which is used as a metallic detergent, for example, for the dispersion of sludge occurring in lubricating oils, the solubilization of a precursor and the neutralization of an acid, especially over-based magnesium sulfonate having a base number of 300 mg-KOH/g or greater in a base stock, in order to improve friction characteristics (see JP Kokai 62-84190). Further, a lubricating oil making combined use of a metallic detergent, such as calcium sulfonate, barium sulfonate or magnesium sulfonate, with a molybdenum dialkyldithiocarbamate was also proposed (see JP Kokai 62-215697).

These metal sulfonates, when employed singly, are however still insufficient in friction reducing effects, so that they are merely friction modifier adjuvants for use in combination with friction modifiers such as phosphate esters and molybdenum dithiocarbamate. If a metal sulfonate having still higher friction reducing ability is identified, it is therefore believed it will find utility in a much wider range of fields and hence to have a significantly-increased industrial value. There is accordingly an outstanding intense desire for the development of such a metal sulfonate.

In view of the circumstances of development of friction modifiers as described above, the present invention has as objects thereof the provision of a novel metal sulfonate having friction reducing ability and also the provision of a lubricating oil composition with the metal sulfonate added.

US-A-4,225,446 claims and describes a process for preparing a fluid, highly basic magnesium sulfonate comprising: (a) forming, in the presence of a volatile solvent, an admixture of an oil-soluble sulfonic acid and a magnesium sulfonate having a total base number in excess of about 200; (b) neutralizing the sulfonic acid; (c) forming a second admixture of (i) the sulfonate prepared from the first admixture, (ii) magnesium oxide, (iii) a naphthenic acid, and (iv) a lower alkanol; (d) treating the second admixture with carbon dioxide; (e) treating the second admixture with (i) water and (ii) ammonia or an ammonium compound during the initial phase of the carbon dioxide treatment; (f) heating the carbonated solution to remove water and the lower alkanol; (g) cooling and thereafter treating the water and lower alkanol depleted solution with additional carbon dioxide; (h) heating the further carbon dioxide treated solution to remove water; and (i) thereafter clarifying the solution.

EP-A-0 312 313 claims and describes an overbased metal sulfonate compound comprising a liquid vehicle and (A) at least one metal alkyl aryl sulfonate containing 1 to 3 alkyl groups, one of which alkyl groups contains an average number of carbon atoms of at least 40 while any remaining alkyl groups contain less than 10 carbon atoms, and (B) at least one metal alkyl aryl sulfonate containing 1 to 3 alkyl groups, one of which alkyl groups contains an average number of carbon atoms of 10 to 33 while any remaining alkyl groups contain less than 10 carbon atoms.

US-A-3,910,994 claims and describes a process for producing an alkylaromatic sulfonate containing a C₉ - C₁₈ linear alkyl group for use as a laundry detergent.

GB-A-2182948 (which is a counterpart of JP Kokai 62-215697 mentioned *supra*) claims and discloses an automatic transmission fluid composition comprising a major amount of a mineral oil and/or synthetic oil as a base oil, and 0.1 - 5% by weight of magnesium sulfonate on the basis of the total amount of the composition as an essential component.

It has been discovered that a metal sulfonate having an alkyl group, which has a specific linear portion determinable by carbon nuclear magnetic resonance (¹³C-NMR measurement) (hereinafter referred to as ¹³C-NMR measurement, as needed), has excellent friction reducing ability. Having been interested in its effectiveness as a friction modifier, it has also been found that its addition to a base stock for lubricating oil makes it possible to furnish a lubricating oil composition having improved friction characteristics and utility in a variety of technical fields. Based on these findings, the present invention has now been completed.

The present invention provides the use for friction reduction of a lubricating oil composition of a metal sulfonate as defined in claim 1 of the set of claims following the description below. The present invention also provides the use as aforesaid in a lubricating composition as defined in claim 5 of the said set of claims. Optional and/or preferred features of the invention are defined in the other claims of the said set of claims.

The metal sulfonatewhich is used as the friction modifier according to the present invention is composed of an organic sulfonic group, which contains a hydrocarbon group, and a metal, and is a compound which can be represented, for example, by the following formula (I):

(RSO₃)ₓM (I)

It may consist of one type of the compound or may be a mixture of two or more compounds having different hydrocarbon groups. In the formula (I), R in the organic sulfonic group RSO₃ is a hydrocarbon group, which is a chain hydrocarbon group or an aromatic group with at least one chain hydrocarbon group bonded thereto. Illustrative of the chain hydrocarbon group can be alkyl groups, each of which has 12-40 carbon atoms on average per organic sulfonic group as measured by ¹³C-NMR and calculated supposing that there is one carbon atom bonded to a sulfonic group. It is particularly preferred to contain at least one or more alkyl groups having 12-30 carbon atoms. Specific examples of the alkyl group can include dodecyl, tridecyl, tetradecyl, pentadecyl, hexadecyl, heptadecyl, octadecyl, nonadecyl, eicosyl, tetracosyl, pentacosyl, hexacosyl, heptacosyl, octacosyl, nonacosyl, triacontyl, pentatriacontyl, and octatriacontyl.

As the metal sulfonate according to the present invention, one having an alkyl chain linearity of 20% or higher, especially of from 30% to 80% as determined by a ¹³C-NMR measurement is preferred.

Here, the term "alkyl chain linearity" is based on a unique concept established by the present inventors as a result of repetition of numerous experiments, and means the ratio of the number of carbon atoms in a linear portion located 5 or more atoms apart from an end of the alkyl group or 4 or more atoms apart from a branched site of the alkyl group to the total number of carbon atoms in the alkyl group. Its value is dependent on the bonding site of an aromatic group and the site of branching of the alkyl group.

In the present invention, the alkyl chain linearity has been determined specifically by the following formula from a ¹³C-NMR measurement.$\text{Alkyl chain linearity (%) =} \frac{\text{Integral intensity over a chemical shift range of from 29 ppm to 31 ppm}}{\text{Sum of all integral intensity over a chemical shift range of from 5 ppm to 60 ppm}} \text{x 100}$

Incidentally, the ¹³C-NMR measurement was conducted by converting the metal sulfonate into its corresponding sulfonic acid.

The present inventors recognized the existence of a correlation between the alkyl chain linearity and the friction reducing effects of its metal sulfonate, and have ascertained that the metal sulfonate exhibits better friction reducing effects as the linearity becomes higher and also that a linearity lower than 20% cannot exhibit the effects fully although a linearity of 20% or higher, especially of from 30% to 80% shows particularly marked effects.

Even when the metal sulfonate contains two or more chain hydrocarbon groups per organic sulfonic group or is a mixture of two or more different compounds (metal sulfonates), the metal sulfonate exhibits friction reducing effects and is effective as a metal sulfonate according to the present invention provided that the alkyl chain linearity as determined by a ¹³C-NMR measurement is 20% or higher. In particular, a metal sulfonate, the chain hydrocarbon groups of which are each an alkyl group having 12 or more carbon atoms and a linearity of 20% or higher, is preferred from the viewpoint of making it possible to substantially increase friction reducing ability. The aromatic group bonded to the chain hydrocarbon groups can be either monocyclic or fused polycyclic. Those represented by the following structural formulas (a) to (g), respectively, are effective, with a phenyl group being particularly preferred.

The metal component represented by M in the above-described metal sulfonate (formula (I)) (RSO₃)ₓM can be an alkali metal or an alkaline earth metal. Further, a metal of an atomic number in a range of from 12 to 56 is also suited. Specific examples can include sodium, potassium, lithium, calcium, magnesium and barium. In addition, aluminum, zinc, tin, chromium, copper, cobalt are also effective. Of these, calcium, magnesium and barium are particularly preferred.

In the above formula (I), x is a value corresponding to the valence of the metal component M.

Typical illustrative compounds of the metal sulfonate according to the present invention can be represented by the following formula (II):

In the above formula (II), A and B may be the same or different and are each (i) an alkyl group or (ii) an aromatic group with at least one alkyl group bonded thereto, and the alkyl groups are those capable of providing 20% or higher as an average linearity of the whole alkyl groups as determined by a ¹³C-NMR measurement. Further, the aromatic group can be at least one aromatic group selected from the group consisting of the above-described structural formulas (a) to (g). In addition, M in the formula represents the above-described divalent metal, with an alkaline earth metal being preferred.

Accordingly, more specific illustrative examples of the metal sulfonate according to the present invention can be represented by the following formulas (III) to (VII):

In the above formulas (III) to (VII), R¹ to R¹⁰ are alkyl groups and as already described, the average total carbon numbers of R¹, R², R³, R⁴, R⁵, R⁶, R⁷, R⁸, R⁹ and R¹⁰, said average total carbon numbers being equivalent to the numbers of carbon atoms per the corresponding organic sulfonic acids, may preferably be from 12 to 40, and R¹ to R¹⁰ have alkyl chain linearities of 20% or higher as determined by ¹³C-NMR measurement.

In each of the above formulas (III) to (VII), each n represents the number of alkyl groups bonded to the associated aromatic group and may stand for an integer of 1 to 5, preferably of 1 to 3. In each formula, two n values can be the same or different.

Further, Ms in the formulas (III) to (VII) are preferably alkaline earth metals, although they can be other divalent metals described above.

No particular limitation is imposed on a process for the preparation of a metal sulfonate according to the present invention, which contains one or more alkyl groups which are large in chain length and high in linearity. It is possible to adopt, for example, a process in which a sulfonic acid available by sulfonation of an alkyl-substituted aromatic hydrocarbon obtained from a petroleum fraction or of an alkyl-substituted aromatic hydrocarbon, which is an alkylation product of an aromatic hydrocarbon by an olefinic hydrocarbon, is neutralized with an alkali metal oxide, hydroxide, alkoxide or the like, followed by the adjustment of a quantity of a metal.

Further, a metal sulfonate according to the present invention, which has a specific alkyl chain linearity, can be prepared by mixing various metal sulfonates of different alkyl chain linearities so that the overall alkyl chain linearity is controlled to fall within the above-descried particular range.

In the present invention, the metal sulfonate can be a basic salt or over-based salt in addition to a neutral salt. Its salt type can be chosen as desired depending on its application. A basic salt can be one prepared by a conventional process, and can be prepared, for example, by dispersing M(OH)₂ or MCO₃ (wherein M represents an alkaline earth metal or the like) in a colloidal form in a sulfonate. A conventionally-adopted preparation process can be relied upon.

As has been described above, the present invention provides a friction modifier, especially a friction modifier for lubricating oils, which is composed of a particular metal sulfonate. This friction modifier is oil-soluble. It can be used by dissolving it in a hydrocarbon or another solvent and diluting the resultant concentrate as needed or as a component of an additive package in combination with other additives.

A description will next be made about the lubricating oil composition according to the present invention.

No particular limitation is imposed on the base stock employed in the lubricating oil composition according to the present invention. The base stock can be any one of mineral base stocks, synthetic base stocks and vegetable base stocks, or can be a blended base stock of two or more of these base stocks.

As a mineral base stock, it is possible to use, for example, a mineral oil obtained by the treatment of a lubricating oil fraction, which is in turn available by vacuum distillation of an atmosphere distillation residue of paraffin-base, neutral or naphthene-base crude oil, through a refining step such as solvent refining, hydrocracking, hydro-refining, catalytic dewaxing, solvent dewaxing or clay treatment; a mineral oil obtained by subjecting a vacuum distillation residue to solvent deasphalting and then treating the resulting deasphalted oil through the above-described refining step; a mineral oil obtained by isomerizing wax components; or a blended oil thereof. In the above solvent refining, an aromatic extraction solvent such as phenol, furfural or N-methylpyrrolidone can be used, whereas as a solvent for the solvent dewaxing, liquefied propane, MEK/toluene, MEK/MIBK, or the like can be used. Among the above-described mineral base stocks, hydro-refined oil is preferred from the standpoint of oxidation stability and the like, and one containing, for example, 2 wt% or less of aromatic hydrocarbons and 90 wt% or more of saturated hydrocarbons can be used.

Examples of synthetic base stocks, on the other hand, can include poly(α-olefin) oligomers of lubricating viscosity; polybutene; alkylbenzenes; polyol esters such as trimethylolpropane esters and pentaerythritol esters; polyoxyalkylene glycols; polyoxyalkylene glycol esters; polyoxyalkylene glycol ethers; dibasic acid esters; phosphate esters; and silicone oils. These base stocks can be used either singly or in combination. Further, usable examples of vegetable base stocks can include rape seed oil, soybean oil, coconut oil, olive oil and sunflower oil.

The lubricating base stock employed in the lubricating oil composition according to the present invention can be produced by suitably preparing a blended base stock so that the blended base stock has properties desired for the intended application of the lubricating oil composition. Concerning viscosity, for example, it is preferred to control the kinematic viscosity at 100°C in a range of from 2 mm²/s to 30 mm²/s, especially from 3 mm²/s to 10 mm²/s for a lubricating oil for internal combustion engines, the kinematic viscosity at 100°C in a range of from 2 mm²/s to 30 mm²/s, especially from 3 mm²/s to 15 mm²/s for an automatic transmission fluid, and the kinematic viscosity at 40°C in a range of from 10 mm²/s to 1,000 mm²/s, especially from 20 mm²/s to 500 mm²/s.

The metal sulfonate according to the present invention can exhibit sufficient friction reducing effects when added to the lubricating base stock in a proportion of from 0.01 to 10 wt%, preferably from 0.05 to 5 wt% based on the whole weight of the lubricating oil composition or in a proportion of from 1 ppm to 10,000 ppm, preferably from 50 ppm to 5,000 ppm in terms of the metal, although the proportion varies depending on the application field of the lubricating oil.

To the lubricating oil composition according to the present invention, it is possible to add selected ones of viscosity index improvers, ashless dispersants, oxidation inhibitors, extreme pressure agents, wear inhibitors, metal deactivators, pour-point depressants, rust inhibitors, other friction modifiers and other additives as needed.

Illustrative usable examples of the viscosity index improvers can include polymethacrylates, polyisobutylenes, ethylene-propylene copolymers, and hydrogenated styrene-butadiene copolymers. These viscosity index improvers are used generally in a proportion of from 3 wt% to 35 wt%.

Illustrative of the ashless dispersants can be polybutenyl-succinimides, polybutenylsuccinamides, benzylamines, and succinate esters. They can be used generally in a proportion of from 0.05 wt% to 7 wt%.

Illustrative examples of the oxidation inhibitors can include amine-type oxidation inhibitors such as alkylated diphenylamines, phenyl-α-naphthylamine and alkylated phenyl-α-naphthylamines; phenolic oxidation inhibitors such as 2,6-di-t-butylphenol and 4,4'-methylene-bis(2,6-di-t-butyl-phenol); and zinc dithiophosphate. They can be used generally in a proportion of from 0.05 wt% to 5 wt%.

Illustrative of the extreme pressure agents can be dibenzyl sulfide and dibutyl disulfide. They can be used generally in a proportion of from 0.05 wt% to 3 wt%.

Illustrative examples of the metal deactivators can include benzotriazole, benzotriazole derivatives, and thiadiazole. They can be used generally in a proportion of from 0.01 wt% to 3 wt%.

Illustrative of the pour-point depressants can be ethylene-vinyl acetate copolymers, chlorinated paraffin-naphthalene condensation products, polymethacrylates, and polyalkylstyrenes. They can be used generally in a proportion of from 0.1 wt% to 10 wt%.

Illustrative of the wear inhibitors can be phosphate esters, zinc thiophosphate, and sulfur compounds. They can be used generally in a proportion of from 0.01 wt% to 5 wt%.

As preferred embodiments of the present invention, it is possible to provide:
(i) A friction modifier for lubricating oils, which comprises a metal sulfonate composed of an organic sulfonic group, which contains a hydrocarbon group, and a metal, in which the hydrocarbon group is a chain hydrocarbon group or an aromatic group with at least one chain hydrocarbon group bonded thereto, and wherein the chain hydrocarbon group is an alkyl group having an average carbon number of from 12 to 40 per organic sulfonic group and an alkyl chain linearity of 20% or higher as determined by a ¹³C-NMR measurement.
(ii) A friction modifier for lubricating oils, which comprises metal sulfonate composed of an organic sulfonic group, which contains a hydrocarbon group, and a metal, in which the hydrocarbon group is a chain hydrocarbon group or an aromatic group with at least one chain hydrocarbon group bonded thereto, and wherein the chain hydrocarbon group is an alkyl group having an average carbon number of from 12 to 40 per organic sulfonic group and has an alkyl chain linearity of 30% or higher as determined by a ¹³C-NMR measurement.
(iii) A lubricating oil composition comprising:
   a lubricating base stock;
   a metal sulfonate composed of an organic sulfonic group, which contains a hydrocarbon group, and a metal, said hydrocarbon group being a chain hydrocarbon group or an aromatic group with at least one chain hydrocarbon group bonded thereto, said chain hydrocarbon group being an alkyl group, which has an average carbon number of from 12 to 40 per organic sulfonic group, and having an alkyl chain linearity of 20% or higher as determined by a ¹³C-NMR measurement, and said metal sulfonate having been added in a proportion of from 1 ppm to 10,000 ppm in terms of the metal thereof based on a whole weight of the lubricating oil composition.
(iv) A lubricating oil composition comprising:
   a lubricating base stock;
   a metal sulfonate composed of an organic sulfonic group, which contains a hydrocarbon group, and a metal, said hydrocarbon group being a chain hydrocarbon group or an aromatic group with at least one chain hydrocarbon group bonded thereto, said chain hydrocarbon group being an alkyl group, which has an average carbon number of from 12 to 40 per organic sulfonic group, and having an alkyl chain linearity of 20% or higher as determined by a ¹³C-NMR measurement, and said metal sulfonate having been added in a proportion of from 1 ppm to 10,000 ppm in terms of the metal thereof based on a whole weight of the lubricating oil composition; and
   at least one additive selected from the group consisting of viscosity index improvers, ashless dispersants, oxidation inhibitors, extreme pressure agents, metal deactivators, pour-point depressants and wear inhibitors.

As a more preferable embodiment of the lubricating oil composition according to the present invention, there is provided a lubricating oil composition comprising as a base stock a hydro-refined oil, which contains 2 wt% or less of aromatic hydrocarbons and 90 wt% or more of saturated hydrocarbons, and a calcium sulfonate containing 1 to 2 C₁₄-₂₄ alkyl groups per organic sulfonic group and having an alkyl chain linearity of 40% or higher as determined by a ¹³C-NMR measurement, said calcium sulfonate having been added in a proportion of from 50 ppm to 5,000 ppm in terms of calcium based on the whole weight of the lubricating oil composition.

As has been described above, the metal sulfonate according to the present invention can be used as a friction modifier in hydraulic working oils, wet brake oils, sliding surface oils, plastic working oils, cutting oils and the like in addition to lubricating oils for internal combustion engines, automatic transmission fluids and gear oils. Without being limited to them, the metal sulfonate can be used without limitations in any other oils insofar as it can exhibit its friction reducing effects.

### Examples

The present invention will next be described specifically by Examples and Comparative Examples. It is however to be noted that the Examples are to primarily demonstrate the unique effects of the alkyl group or groups in the metal sulfonate according to the present invention and that the present invention shall not be limited by these Examples.

The alkyl chain linearities of the metal sulfonates employed in the following Examples and the performance evaluation of the lubricating oil compositions were measured or conducted by the following methods.

### (i) Measuring method of alkyl chain linearity

Each metal sulfonate was converted into its corresponding sulfonic acid, and under the following measuring conditions, its ¹³C-NMR spectrum was measured. Further, its alkyl chain linearity was calculated in accordance with the below-described formula.

| Measuring conditions | |
|---|---|
| Used instrument | EX400 (manufactured by JEOL Ltd.) |
| Observed nucleus | ¹³C |
| Observing frequency | 100.50 MHz |
| Measuring mode | Inverse gated ¹H decoupling |
| Internal standard | TMS (= 0 ppm) |
| Relaxation reagent | Cr(acac)₃ |
| Solvent | CDCl₃ |
| Quantity of sample | 300 mg |
| Temperature | 30°C |

$\text{Alkyl chain linearity (%) =} \frac{\text{Integral intensity over the chemical shift range of from 29 ppm to 31 ppm}}{\text{Sum of all integral intensity over the chemical shift range of from 5 ppm to 60 ppm}} \text{x 100}$

### (ii) Performance evaluation

### Measuring method of friction coefficients

Concerning lubricating oil compositions with corresponding metal sulfonates added in predetermined proportions, their friction coefficients were measured under the following conditions by using "LFW-1" as a testing machine.

| Friction materials | steel/steel |
|---|---|
| Load | [200 lb.] 90.718 kg |
| Oil temperature | 80°C |
| Revolution speed | 600 rpm |
| Measuring period | 30 minutes |

### Example 1

Provided was Calcium Sulfonate I of the following characteristics:
- Average number of alky 1 carbons per organic 31 sulfonic group
- Alkyl chain linearity 47.2%
- Calcium content 2.8 wt%
- Total base number 25 mg-KOH/g

A lubricating oil composition was formulated by adding the sulfonate to a solvent-refined mineral oil "100N" (kinematic viscosity at 100°C: 4.2 mm²/s) in a proportion of 140 ppm in terms of calcium based on the whole weight of the lubricating oil composition. The friction coefficient of the resultant lubricating oil composition was measured by the above-described method. It was found to be 0.09.

### Example 2

A lubricating oil composition was formulated in exactly the same manner as in Example 1 except that the proportion of Calcium Sulfonate 1 was increased from 140 ppm to 560 ppm in terms of calcium. The resultant lubricating oil composition was subjected to a performance evaluation. Its friction coefficient was found to be 0.08, thereby indicating an improvement in friction characteristics.

### Example 3

Provided was Calcium Sulfonate 2 of the following characteristics:
- Average number of alky 1 carbons per 35 organic sulfonic group
- Alkyl chain linearity 39.9%
- Calcium content 12 wt%
- Total base number 300 mg-KOH/g

A lubricating oil composition was formulated by adding the sulfonate to the same lubricating base stock as that employed in Example 1 in a proportion of 1,200 ppm in terms of calcium based on the whole weight of the lubricating oil composition. The resultant lubricating oil composition was subjected to the above-described performance evaluation. Its friction coefficient was found to be 0.10.

### Example 4

A lubricating oil composition was formulated in exactly the same manner as in Example 3 except that the proportion of Calcium Sulfonate 2 was increased from 1,200 ppm to 2,400 ppm in terms of calcium. The resultant lubricating oil composition was subjected to a performance evaluation. Its friction coefficient was found to be 0.08.

### Example 5

Provided was Calcium Sulfonate 3 of the following characteristics:
- Average number of alky 1 carbons per 26 organic sulfonic group
- Alkyl chain linearity 31.0%
- Calcium content 11.8 wt%
- Total base number 295 mg-KOH/g

A lubricating oil composition was formulated by adding the sulfonate to the same lubricating base stock as that employed in Example 1 in a proportion of 2,400 ppm in terms of calcium based on the whole weight of the lubricating oil composition. The resultant lubricating oil composition was subjected to the above-described performance evaluation. Its friction coefficient was found to be 0.09.

### Example 6

A lubricating oil composition was formulated in exactly the same manner as in Example 5 except that the proportion of Calcium Sulfonate 3 was increased from 2,400 ppm to 4,800 ppm in terms of calcium. The resultant lubricating oil composition was subjected to a performance evaluation. Its friction coefficient was found to be 0.08.

### Comparative Example 1

Provided was Calcium Sulfonate 4 of the following characteristics:
- Average number of alkyl carbons per 33 organic sulfonic group
- Alkyl chain linearity 17.2%
- Calcium content 12 wt%
- Total base number 300 mg-KOH/g

A lubricating oil composition was formulated by adding the sulfonate to the same lubricating base stock as that employed in Example 1 in a proportion of 2,400 ppm in terms of calcium based on the whole weight of the lubricating oil composition. As a result of a performance evaluation, its friction coefficient was found to be 0.13.

### Comparative Example 2

Provided was Calcium Sulfonate 5 of the following characteristics:
- Average number of alky 1 carbons per 31 organic sulfonic group
- Alkyl chain linearity 12.6%
- Calcium content 11.7 wt%
- Total base number 295 mg-KOH/g

A lubricating oil composition was formulated by adding the sulfonate to the same lubricating base stock as that employed in Example 1 in a proportion of 2,400 ppm in terms of calcium based on the whole weight of the lubricating oil composition. The friction coefficient of the resultant lubricating oil composition was found to be 0.14.

### Comparative Example 3

A lubricating oil composition was formulated in exactly the same manner as in Comparative Example 2 except that the proportion of Calcium Sulfonate 5 was increased from 2,400 ppm to 4,800 ppm in terms of calcium. Its friction coefficient was found to be 0.13. The calcium sulfonate, the alkyl chain linearity of which is low, was also found to be unable to bring about any substantial advantageous effects on friction characteristics despite the increase in its proportion.

### Comparative Example 4

The solvent-refined mineral oil "100N" (kinematic viscosity at 100°C: 4.2 mm²/s), which was employed as a lubricating base stock in Example 1, was subjected by itself to a performance evaluation. Its friction coefficient was found to be 0.14.

The measurement results of the friction coefficients in the above Examples and Comparative Examples and the calcium sulfonates employed therein are summarized in Table 1 and Table 2, respectively. From these results, it is appreciated that an alkyl chain linearity of 20% or higher in a metal sulfonate provides a low friction coefficient even if the metal sulfonate is added in a small proportion (Examples 1 and 2) whereas a lower alkyl chain linearity cannot provide a low friction coefficient even if the proportion of the metal sulfonate is increased (Comparative Example 3). From a comparison between Comparative Example 2 and Comparative Example 4, it is indicated that use of a metal sulfonate having a linearity lower than 20% results in a lubrication oil composition the friction coefficient of which is the same as that of the base stock alone. It has therefore been elucidated that the alkyl chain linearity is a primary element governing friction characteristics.

From this it is readily seen that a metal sulfonate having an alkyl chain linearity of 20% or higher is useful as a friction modifier for lubricating oils, and can improve the friction characteristics of lubricating oil compositions.

## Claims

1. The use for friction reduction of a lubricating oil composition of a metal sulfonate composed of a metal and an organic sulfonic group which contains a hydrocarbon group, wherein the hydrocarbon group is a chain hydrocarbon group or an aromatic group with at least one chain hydrocarbon group bonded thereto, said chain hydrocarbon group having an alkyl chain linearity of 20% or higher as determined by a carbon nuclear magnetic resonance measurement (¹³C-NMR measurement).

2. Use of claim 1, wherein said chain hydrocarbon group is an alkyl group.

3. Use of claim 1 or claim 2 wherein said chain hydrocarbon group is one or more alkyl groups each of which has 12 to 40 carbon atoms on average per organic sulfonic group as determined by ¹³C-NMR measurement.

4. Use as in any one of claims 1 to 3 wherein the chain hydrocarbon group has an alkyl linearity of 30% to 80% as determined by ¹³C-NMR measurement.

5. Use as in any one of claims 1 to 4 in a lubricating oil composition comprising a base stock, wherein the metal sulfonate is added to the composition in an amount to provide from 1ppm to 10,000ppm in terms of the metal thereof based on the total weight of the lubricating oil composition.

6. Use as in any one of claims 1 to 5 wherein the lubricating oil composition comprises at least one additive selected from viscosity index improvers, ashless dispersants, oxidation inhibitors, extreme pressure agents, metal deactivators, pour point depressants, and wear inhibitors.

## Patentansprüche

1. Verwendung einer Schmierölzusammensetzung von Metallsulfonat, das aus Metall und organischer Sulfongruppe zusammengesetzt ist, die eine Kohlenwasserstoffgruppe enthält, wobei die Kohlenwasserstoffgruppe eine Ketten-Kohlenwasserstoffgruppe oder ein aromatische Gruppe mit mindestens einer daran gebundenen Ketten-Kohlenwasserstoffgruppe ist, wobei die Ketten-Kohlenwasserstoffgruppe eine Alkylkettenlinearität von 20 % oder höher hat, bestimmt mittels Kohlenstoff-Kernresonanzmessung (¹³C-NMR-Messung), zur Reibungsverminderung.

2. Verwendung nach Anspruch 1, bei der die Ketten-Kohlenwasserstoffgruppe eine Alkylgruppe ist.

3. Verwendung nach Anspruch 1 oder Anspruch 2, bei der die Ketten-Kohlenwasserstoffgruppe eine oder mehrere Alkylgruppen ist, die jeweils durchschnittlich 12 bis 40 Kohlenstoffatome pro organischer Sulfongruppe haben, bestimmt mittels ¹³C-NMR-Messung.

4. Verwendung nach einem der Ansprüche 1 bis 3, bei der die Ketten-Kohlenwasserstoffgruppe eine Alkyllinearität von 30 % bis 80 % hat, bestimmt mittels ¹³C-NMR-Messung.

5. Verwendung nach einem der Ansprüche 1 bis 4 in einer Schmierölzusammensetzung, die Basismaterial umfasst, wobei das Metallsulfonat der Zusammensetzung in einer Menge zugefügt wird, um 1 ppm bis 10.000 ppm in Form seines Metalls zu liefern, bezogen auf das Gesamtgewicht der Schmierölzusammensetzung.

6. Verwendung nach einem der Ansprüche 1 bis 5, bei der die Schmierölzusammensetzung mindestens ein Additiv ausgewählt aus Viskositätsindexverbesserern, aschefreien Dispergiermitteln, Oxidationsschutzmitteln, Extremdruckmitteln, Metalldesaktivatoren, Stockpunktsenkungsmitteln und Verschleißschutzmitteln umfasst.

## Revendications

1. Utilisation pour une réduction de frottement d'une composition d'huile lubrifiante d'un sulfonate de métal composé d'un métal et d'un groupe sulfonique organique qui contient un groupe hydrocarboné, dans laquelle le groupe hydrocarboné est un groupe hydrocarboné en chaîne ou un groupe aromatique avec au moins un groupe hydrocarboné en chaîne qui lui est relié, ledit groupe hydrocarboné en chaîne ayant une linéarité de chaîne alkyle de 20% ou plus, comme déterminé par une mesure de résonance magnétique nucléaire du carbone (mesure du ¹³C-RMN).

2. Utilisation selon la revendication 1, dans laquelle ledit groupe hydrocarboné en chaîne est un groupe alkyle.

3. Utilisation selon la revendication 1 ou la revendication 2, dans laquelle ledit groupe hydrocarboné en chaîne est formé d'un ou plusieurs groupes alkyle, dont chacun a 12 à 40 atomes de carbone en moyenne par groupe sulfonique organique, comme déterminé par mesure du ¹³C-RMN.

4. Utilisation selon l'une quelconque des revendications 1 à 3, dans laquelle le groupe hydrocarboné en chaîne a une linéarité d'alkyle de 30% à 80%, comme déterminé par mesure du ¹³C-RMN.

5. Utilisation selon l'une quelconque des revendications 1 à 4 dans une composition d'huile lubrifiante comprenant une base, dans laquelle le sulfonate de métal est ajouté à la composition en quantité telle qu'il y ait 1 ppm à 10 000 ppm qui y soient présents en termes de métal par rapport au poids total de la composition d'huile lubrifiante.

6. Utilisation selon l'une quelconque des revendications 1 à 5, dans laquelle la composition d'huile lubrifiante comprend au moins un additif choisi parmi les agents promoteurs d'indice de viscosité, les dispersants sans cendres, les inhibiteurs d'oxydation, les agents de pressions extrêmes, les désactivateurs de métaux, les agents réducteurs du point d'écoulement et les inhibiteurs d'usure.
